

March 25, 1924.

1,488,186

J. H. YOUNG

BUILDING MATERIAL

Filed Jan. 28, 1922

Fig. 1.



Fig. 2.



Fig. 3.



Fig. 4.



Fig. 5.

Inventor:  
James Howard Young  
by Jas. H. Lohmehill  
atty.

## UNITED STATES PATENT OFFICE.

JAMES HOWARD YOUNG, OF PITTSBURGH, PENNSYLVANIA, ASSIGNOR TO H. H. ROBERTSON COMPANY, OF PITTSBURGH, PENNSYLVANIA, A CORPORATION OF PENNSYLVANIA.

## BUILDING MATERIAL.

Application filed January 28, 1922. Serial No. 532,403.

*To all whom it may concern:*

Be it known that I, JAMES HOWARD YOUNG, a citizen of the United States, residing in Pittsburgh, in the county of Allegheny and State of Pennsylvania, have invented an Improvement in Building Material, of which the following description, in connection with the accompanying drawings, is a specification, like characters on the drawings representing like parts.

This invention relates to an improved article of manufacture having an exterior metal surface which is affixed to a flexible non-metallic foundation or underlying member by a layer of asphalt or like bituminous material. The foundation member is flexible and of non-metallic material, such as felt, paper or fabric, which is coated or saturated with asphalt or like bituminous material, and in accordance with this invention is provided with an exterior surface or coating of metal, preferably lead, zinc, copper or like so-called non-corrodible metals, which metal surface is composed of a layer of finely divided metal particles which are embedded in the asphaltic layer, and an additional layer of finely divided metal particles which are molecularly united with the metal particles embedded in the asphaltic layer.

The finely divided particles of metal forming the layer which is embedded in the asphalt layer are formed by spraying or projecting molten metal upon and into the asphalt layer, and the finely divided particles forming the metallic layer which is molecularly united with the first mentioned metallic layer are also formed from molten metal and are projected against the embedded particles under sufficient pressure to weld or molecularly unite the metal particles of both layers while said particles are in a heated condition and thus provide the flexible fibrous layer with a metal surface or coating of substantially uniform thickness, which conforms to the contour of the bituminous covered fibrous article and does not detrimentally impair the flexibility of the fibrous layer, so that the fibrous layer with the metallized surface adhesively affixed thereto by the bituminous material may be rolled into convenient form for shipping and for applying the same to a roof, floor, siding or the like.

55 The metal coating or surface may be made

of any desired thickness, as succeeding layers of metal particles may be projected upon and molecularly united with the underlying layer of metal particles.

The metal coating or surface may be made 60 of a sufficient number of molecularly united layers to provide a non-porous coating or surface upon the asphalt layer, but it may be preferred to employ a relatively thin metal coating or surface which is more or 65 less porous, as by so doing provision is made for the escape of the volatile ingredients in the asphalt and blistering of the metal coating is thereby prevented.

The underlying layer of non-metallic 70 fibrous material may be made of material length and wound into the form of a roll, or it may be of shorter lengths in the form of a sheet or strip, or it may be made of still shorter lengths and substantially in the form 75 of a shingle.

These and other features of this invention will be pointed out in the claims at the end of this specification.

Fig. 1 represents a roll of flexible fibrous 80 material embodying this invention.

Fig. 2 a developed view of a portion of the roll shown in Fig. 1, parts of the layers being omitted.

Fig. 3, an enlarged cross section on the 85 line 3—3, Fig. 2.

Fig. 4, a plan of a shingle embodying the invention, parts of the layers being omitted, and

Fig. 5, a plan illustrating a plurality of 90 shingles made from a sheet or strip embodying the invention.

Referring to the drawing, *a* represents the article or underlying layer to be protected, which as above stated is composed of flexible fibrous material, such as fabric, felt, paper and the like, which is covered on one or both surfaces with a layer *b* of asphalt or like bituminous material, or which is impregnated with the asphalt.

In the present instance the fibrous layer *a* is enveloped by the asphalt layer *b*, and the latter is provided with a protective metal coating composed of a plurality of layers of finely divided metal, such as lead, 95 zinc, copper and the like, and in the present instance two layers *c*, *d* are herein represented.

The metal layers *c*, *d*, are composed of finely divided metal particles 10, 12, re- 110

spectively, which are formed by spraying or projecting molten metal upon the asphalt coated layer *a* with any suitable apparatus, as for instance, substantially that shown and described in U. S. Patent No. 495,107 dated April 11, 1893. The finely divided metal particles are projected against the asphalt coated fibrous sheet or layer *a* while the asphalt coating is in a more or less tacky or yielding condition and preferably soon after the asphalt coating has been applied to the fibrous sheet or layer *a*, with the result that the metal particles 10, which strike against the asphalt layer *b* penetrate into 15 and are embedded in the asphalt layer, and as they encounter a minimum resistance, they retain their original shape, which for sake of distinction, is represented in Fig. 2 as round or spherical, and thus form the 20 underlying or embedded layer *c*.

On the other hand, the metal particles 12 which are projected while hot against the layer *c* of embedded metal particles while the latter are in a heated condition strike 25 the same with force sufficient to cause the heated metal particles to cohere at their contacting points or surfaces and become welded or molecularly united and form the metal layer *d*, which is thus molecularly 30 united or welded to the underlying or embedded metal layer *c*.

The metal particles 12 comprising the overlying or exterior layer *d*, are more or less distorted or changed from their original 35 shape by impact against the particles of the underlying layer *c*, and this change or distortion is represented by the irregular or other than round shape of the particles comprising the exterior or surface layer as represented in Fig. 2.

It is evident that by going over the asphalt covered sheet or layer *a* with the finely divided metal particles while the latter are hot a sufficient number of times or by going 45 over the asphalt coated sheet or layer slowly enough a plurality of layers *d* may be built upon the embedded layer *c*, to provide the asphalt coated sheet *a* with a non-porous metal coating composed of the underlying 50 embedded layer *c* and a plurality of overlying or welded layers *d*, but it is preferred to provide the asphalt coated sheet or layer *a* with a metal coating which is more or less porous for two purposes, to wit, 55 to prevent blistering as above described and to economize in the cost of the protected sheet, which result may be obtained with a single metal layer *d* welded to the embedded layer *c*.

The exterior metal surface or coating is 60 firmly affixed to the asphalt coated sheet *a* and a highly efficient article is obtained, which is especially useful for building purposes, and more particularly for roofing and 65 siding purposes, as the underlying sheet or

layer *a* may be made of fibrous material such as asbestos felt or paper, fabric or the like, which is capable of being wound into the form of a roll as represented in Fig. 1, in which form it can be shipped to the job and 70 unwound with the metal surface on the outside, without liability of the metal coating being detached from the asphalt coated sheet or layer of fibrous material, as the asphalt coating may be of such character or quality as to possess the flexibility desired to 75 retain a firm grip upon the embedded particles of the metal coating and thus permit the protected sheet or layer to be rolled up and unrolled, without permitting or causing 80 separation of the metal coating from the asphalt coated sheet or layer *a*.

The asphalt coated sheet or layer *a* of fibrous material having the metal exterior surface or coating *d* may be made and 85 shipped in the form of a roll as represented in Fig. 1, and unrolled into flat form, represented in Fig. 2, or it may be made in shorter lengths and provided with tabs 20 as shown in Fig. 5 to represent a series of connected shingles, or it may be made in still shorter lengths and in the form of individual shingles as represented in Fig. 4.

The metallized flexible fibrous product herein shown possesses advantages over the ordinary rolled roofing, in that it is provided with a metal exterior surface which is affixed to the underlying fibrous layer so as to form a practically permanent metal surface therefor, which is continuous and can be rolled up without liability of being separated therefrom and which is fire and weather resisting, does not disintegrate under the influence of the weather and which can be painted in any color. By the term 100 "asphalt" as used in the claims, it is desired to include pitch or like bituminous or hydrocarbonaceous material.

#### Claims:

1. An improved article of manufacture composed of an underlying member of fibrous material having a layer of asphalt thereon and having a metal coating for said asphalt layer comprising a layer of metal particles embedded in said asphalt layer and a layer of metal particles molecularly united with the particles of said embedded layer.

2. An improved article of manufacture composed of a flexible underlying member of fibrous material having a layer of asphalt thereon and having a metal coating for said asphalt layer comprising a layer of metal particles embedded in said asphalt layer and a layer of metal particles molecularly united with the particles of said embedded layer.

In testimony whereof, I have signed my name to this specification.

JAMES HOWARD YOUNG,